

(Model.)

F. WOOLFENDEN & H. L. O'BRIEN.

MANTEL AND FRONT.

No. 269,772.

Patented Dec. 26, 1882.



Witnesses:

W. B. Masson

Wm. Turner

Inventors

F. Wolfenden

H. L. O'Brien

Per T. J. W. Robertson

Attorney

# UNITED STATES PATENT OFFICE.

FREDERICK WOOLFENDEN AND HERBERT L. O'BRIEN, OF DETROIT, MICH.

## MANTEL AND FRONT.

SPECIFICATION forming part of Letters Patent No. 269,772, dated December 26, 1882.

Application filed February 20, 1882. (Model.)

*To all whom it may concern:*

Be it known that we, FREDERICK WOOLFENDEN and HERBERT L. O'BRIEN, of Detroit, in the county of Wayne and State of Michigan, have invented new and useful Improvements 5 in Mantels and Fronts; and we do hereby declare that the following is a full, clear, and exact description thereof, reference being had to the accompanying drawings, which form a part 10 of this specification.

The nature of our invention relates to certain new and useful improvements in the construction of mantels and the fronts which support them.

15 The invention consists in constructing such mantels and supports as are usually found in dwellings of paper or fiber pulp, as more fully hereinafter described.

In the accompanying drawing is shown an 20 ordinarily-shaped mantel and front. This is made of paper or fiber pulp pressed into shape

in suitable molds, which will allow any desired form or ornamentation to be given to them. After being thus pressed into shape the mantel and front is dried and lacquered or given any 25 other finish desired.

The mantel and front may be made in one piece, or in several pieces, to be afterward joined together, if desired. The latter course would in some instances be preferable where 30 the article must be packed and shipped to a distance from the place of production.

What we claim as our invention is—

As a new article of manufacture and sale, a mantel and front made of paper or fiber pulp 35 pressed in molds, substantially as described.

FREDERICK WOOLFENDEN.  
HERBERT L. O'BRIEN.

Witnesses:

GEO. R. WOOLFENDEN,  
A. S. AUSTIN.